

97

89,311



GEORGE HEIM, OF NAPERVILLE, ILLINOIS, ASSIGNOR TO HIMSELF AND JOHN RUCHTY,  
OF SAME PLACE.

Letters Patent No. 89,311, dated April 27, 1869.

IMPROVED COMPOUND FOR FORMING BUILDING-BLOCS.

The Schedule referred to in these Letters Patent and making part of the same.

To all whom it may concern:

Be it known that I, GRORGE HEIM, of Naperville, in the county of Du Page, and State of Illinois, have invented a new and useful compound for building-purposes; and I do hereby declare the following to be a full, clear, and exact description of the same.

The nature of my invention consists in taking the ingredients hereafter specified, and simply mixing them together, and putting in water enough to make the mixture of the plastic state of ordinary mortar used by plasterers.

The mixture, or compound thus formed is then moulded in blocks, of any suitable size or shape for any desired purposes, or it may be spread on a roof, to form an outside coat, or it may be plastered upon the outside of a house-wall which has been previously lathed, or put in any other place where it is desirable to have a hard, impervious coating. When the compound thus formed becomes dry, it becomes extremely hard, and is highly impervious to the action of the elements, which tend to destroy the ordinary prepared building-material.

To enable those skilled in the art to understand how to manufacture and use my invention, I will proceed to describe the same with particularity.

To one part of stone-lime and one part of water-lime, ~~cement~~, I add from four to eight parts of ~~cement~~ coal-ashes and coal-dust, mixed in about equal quantities, and, to this mixture, I add about two pounds of potash to each bushel of cement used. I then add water till the mixture is reduced to about the consistency of ordinary mortar used for plastering-purposes, stirring the same while the water is being added, in order that the different ingredients may be well mixed together.

The mixture is moulded or applied for use when it is in this plastic state, and left to dry.

The quantity of coal-ashes and coal-dust used, in proportion to the quantity of lime and cement, depends upon the quality of the lime.

Having thus described the nature and use of my invention,

What I claim, and desire to secure by Letters Patent, is—

A compound for building-purposes, manufactured substantially as herein described.

GEORGE HEIM.

Witnesses:

CHENEY M. CASTLE,  
ALVIN SCOTT.